

Aug. 17, 1943.

W. W. DE LAMATTER

2,327,097

METHOD OF TREATING TWISTER GEARS FOR WIRE FABRIC-MAKING MACHINES

Filed Jan. 25, 1940

FIG. 1.



FIG. 2.



FIG. 3.



FIG. 4.



FIG. 5.



FIG. 6.



Inventor:

William W. De Lamatter,  
by: John E. Jackson  
his Attorney.

## UNITED STATES PATENT OFFICE

2,327,097

METHOD OF TREATING TWISTER GEARS  
FOR WIRE FABRIC-MAKING MACHINES

William W. De Lamatter, Cleveland, Ohio, assignor to The American Steel and Wire Company of New Jersey, a corporation of New Jersey

Application January 25, 1940, Serial No. 315,591

4 Claims. (Cl. 76—101)

This invention relates to twister gears for wire fabric-making machines, the objects being to effectively recondition worn twister gears and to provide twister gears which will not wear out as rapidly as conventional twister gears. Other objects and advantages will become apparent from the following disclosure.

A twister gear of the above character is made with a toothed periphery interrupted by a slot extending radially to the axis of the gear or slightly beyond. This slot is adapted to receive two or more wires which are then intertwined upon rotation of the gear. The metal of the twister gear wears rapidly at the bottom of the slot because this is where the wires bear while they are being intertwined, the remainder of the slot functioning only to guide the wires to the slot bottom. Heretofore, a twister gear was discarded when it became worn in this manner.

According to the present invention, such a worn twister gear is first annealed in a furnace at about 2100° Fahrenheit in a reducing atmosphere, for about 15 minutes, this giving the gear a bright anneal. After being so heated for this 15 minute period, it is removed and placed in a cooling chamber where it is kept for about 30 minutes, this cooling chamber also being supplied with a reducing atmosphere and the gear there cooling to below its oxidation point, whereby it comes out bright.

Next, a hole is drilled axially through the gear, this hole being about  $\frac{1}{4}$  of an inch in diameter so that the drilling serves to remove all of the worn metal surrounding the bottom of the gear slot. Then a cylindrical tantalum carbide insert, approximately  $\frac{1}{4}$  of an inch in diameter and about .16 of an inch high, is press-fitted into the hole drilled through the gear. This insert has a rough radial slot opening from its periphery and extending to or beyond its axis, and this slot is, in each instance, aligned with the remaining portion of the gear slot remaining after the drilling.

A curved piece of copper wire in the form of a curl of about the same diameter as the diameter of the hole drilled through the gear, is now tied in the hole of the gear so it covers the juncture between the insert and the gear, the tying being done by means of a loop of stainless steel wire bent around the bottom of the slot of the insert and the opposite periphery of the gear. The curl of copper wire serves as brazing metal, and it is necessary that the gear, the insert and the copper wire be perfectly clean and free from oxides or grease.

Brazing is effected by placing the gear in a brazing furnace, the gear being positioned with the copper curl uppermost. In the brazing furnace, the gear is heated to approximately 2100° Fahrenheit for about 15 minutes, the copper wire melting during this time and running down so as to completely fill all of the space between the press-fitted parts of the insert and the gear. The gear is subsequently placed in a cooling chamber until it cools to a nonoxidizing temperature, both the brazing furnace and this cooling chamber being provided with a reducing atmosphere so that the gear comes out bright.

It is the inventor's opinion that the brazed joint provided by the above procedure results in a metal juncture comprising alloys of copper and iron and of copper and tantalum carbide. However, regardless of the correctness of this opinion, the insert is permanently fixed in the hole drilled in the gear and there is no unfilled space between the insert and the gear at any point.

Upon cooling sufficiently, the stainless steel tie wire is cut off, it being understood that the temperature to which the gear is heated is insufficient to result in melting of either the gear or stainless steel tie wire.

At this time, the gear is carburized in a molten cyanide salt bath where it is kept at a temperature of about 1500° to 1600° Fahrenheit for one or two hours. Upon completion of this carburizing treatment, the gear is quenched in water, this leaving the gear case-hardened to a hardness of from 50 to 55 C. Rockwell.

Ultimately, the case-hardened gear is further treated by lapping or polishing the metal bounding its slot, this being done either with a copper disk using an abrasive powder, such as boron carbide or diamond dust, or by means of a rubber wheel impregnated with diamond grit. Since there is no space between the insert and the gear, this operation results in a perfectly continuous and polished surface on either side of the gear slot.

The foregoing is illustrated by the accompanying drawing, in which:

Figure 1 is a front view of a worn twister gear;

Figure 2 shows the same with the hole drilled;

Figure 3 shows the same with the insert in place and the brazing metal tied;

Figure 4 is a section taken from the line IV—IV in Figure 3;

Figure 5 shows the insert braced in place with tie removed, and

Figure 6 shows the final result.

More specifically, the drawing shows a conventional twister gear with its journals 1, peripheral teeth 2, and a wire receiving slot 3, it being the bottom of this slot which becomes worn in the case of an old gear and which is most apt to wear in the case of a new gear.

In Figure 2, the gear is shown as it appears after the hole is drilled, the hole being shown at 4. Next, Figures 3 and 4 show the twister gear with a tantalum carbide insert pressed in place in the hole and with the copper curl 5 tied in place by means of a loop of stainless steel wire 6. After the brazing step and the removal of stainless steel tie wire, the gear appears as shown by Figure 5, the brazed joint being indicated at 7. The finished gear appears as shown by Figure 6, it now being case-hardened by cyaniding and the bounding walls of the slot finished by grinding and polishing, as required.

I claim:

1. A method of treating a twister gear for a wire fabric-making machine, including forming a hole axially through the gear, placing a hard metal insert in this hole and fixing the insert permanently in the hole by placing a curved wire at the juncture of the insert and gear, tying this curved wire in place with wire having a higher melting temperature than the curved wire and heating the gear to a temperature above the melting temperature of the curved wire and below the melting temperature of the tying wire.

2. A method of reconditioning a wire fabric-making machine twister gear that is worn at the bottom of its slot, including removing metal surrounding the slot bottom to provide an opening, placing an insert having a radial slot in this opening, aligning its slot with the remainder of the twister gear slot, and cementing this insert permanently in place with metal.

3. A method of treating a wire fabric-making machine twister gear, comprising drilling a hole axially through said gear to remove metal surrounding the gear slot bottom, press-fitting a metal carbide cylindrical insert having a radial slot into said hole with its slot aligned with the remainder of the gear slot, tying a curved copper wire in said hole on said insert at the juncture of the two with stainless steel wire, placing said gear in a furnace so as to heat the same to a temperature above the melting temperature of copper and below the melting temperature of stainless steel and of the gear metal, and subsequently grinding and polishing the complete gear slot as required to obtain a satisfactory finish.

4. A method of treating a wire fabric-making machine twister gear, comprising drilling a hole axially through said gear to remove metal surrounding the gear slot bottom, press-fitting a metal carbide cylindrical insert having a radial slot into said hole with its slot aligned with the remainder of the gear slot, tying a curved wire in said hole on said insert at the juncture of the two with stainless steel wire, placing said gear in a furnace so as to heat the same to a temperature above the melting temperature of copper and below the melting temperature of stainless steel and of the gear metal, and subsequently grinding and polishing the complete gear slot as required to obtain a satisfactory finish, said gear being positioned in said furnace with said copper wire uppermost so the melting copper runs down into the space between the press-fitted portions of said insert and gear, whereby the complete gear slot has continuous surfaces.

WILLIAM W. DE LAMATTER.